

## UNITED STATES PATENT OFFICE

2,524,625

## METHOD OF MAKING SHAPED SYNTHETIC PRODUCTS

Nicolas Drisch and Rene Fays, Paris, France, assignors to Comptoir des Textiles Artificiels, a corporation of France

No Drawing. Application February 23, 1946, Serial No. 649,778. In France May 25, 1943

Section 1, Public Law 690, August 8, 1946  
Patent expires May 25, 1963

2 Claims. (Cl. 18—54)

1

This invention relates to a new and improved method of producing synthetic products. More particularly, it relates to a new and improved method of making shaped synthetic structures, such as yarns, threads, filaments, bristles, foils, caps, bands and the like.

In the development of synthetic yarns and related products derived from cellulose, there has been a progressive improvement in the properties of the products, rendering them more and more similar to the natural products. In some cases, the synthetic products have even surpassed the natural products.

One of the serious defects of synthetic yarns, and especially regenerated cellulose products, is their considerable loss of strength on wetting with water. In general, regenerated cellulose yarns lose one-half their strength on wetting with water. It is true that the tensile strength of wool also diminishes on wetting with water, but the tensile strength of cotton, instead of decreasing, increases slightly under such conditions. Wetting, in addition to reducing the tensile strength of regenerated cellulose yarns, also produces considerable swelling which is considerably greater than that of cotton yarn and other yarns formed of natural fibers. The swelling of regenerated cellulose yarn by water is of the order of 100% or more, expressed as the weight of water absorbed by the dry material, whereas it is of the order of 30% for cotton. This swelling considerably reduces the tensile strength and resistance to friction (which is moreover also affected for other reasons) of regenerated cellulose yarns. It also decreases the resistance to chemical agents, particularly to alkalis and acids. Synthetic yarns, and especially those of regenerated cellulose, also differ from yarns of natural fibers in that the former are wetted very rapidly. A sample of ordinary viscose fiber will be immersed in water much more rapidly than a sample of wool, and drops of water falling on a fabric of viscose rayon yarn are absorbed almost immediately, whereas in a wool fabric (having exactly the same structure and the same surface composition) the drops do not spread but slide along the fabric. The explanation of this phenomenon must be sought in the changes produced by the treatments which the initial cellulosic material undergoes during the course of manufacturing the synthetic yarns. The initial cellulosic material is a high polymer composed of bundles of long-chained molecules arranged more or less parallel to the axes of the fibers. This molecular and supermolecular structure is

2

destroyed to a great extent in order to permit dissolution of the cellulose material. To convert the solution into yarn under practical conditions, the solution must have certain properties which can only be acquired by degradation of the molecular chain, that is, by more or less shortening the chains. In spinning the solutions finally obtained, attempts are made to reconstruct orientated structures, that is, to create a new organization of cellulosic chains which were harshly treated by the different treatments to which they were subjected. The structures thus obtained differed considerably from those present in the initial material. The obtained structures contain a large number of strongly polar hydroxyl groups having a great affinity for water. The presence of many more polar groups in the synthetic yarns (particularly in regenerated cellulose yarns but more generally in all products obtained from solutions of cellulosic material or its derivatives) than in natural products explains the special behavior of the synthetic products in the presence of water.

Attempts have been made for a long time to 25 eliminate the aforementioned defects in synthetic products (obtained from solutions of cellulosic materials containing free hydroxyl groups by spinning, molding, etc.), such as yarns, continuous filaments, fibers, bristles, foils, casings, tubings, caps, bands, etc., by blocking the free hydroxyl groups in the regenerated cellulose by one of the following processes:

(a) physical association of regenerated cellulose with ordinary resins or other hydrophobic material, either by introduction into the spinning solution, etc. or by incorporation into the yarn, the resins forming coatings or inert masses within the product and without reacting with the cellulose;

(b) substitution of the free hydroxyl groups in regenerated cellulose by esterification, etherification, etc., or in general by hydrophobic groups;

(c) blocking the hydroxyl groups in regenerated cellulose with the formation of bridges between the chains, thereby increasing the general strength of the cellulosic structure.

The treatment of cellulosic substances containing free hydroxyl groups with formaldehyde or formaldehyde-producing substances, and known as "stenosation," has been studied to a great extent both theoretically and practically. It is generally believed that stenosation leads to the formation of methylene cellulose where the methylene group combines with two hydroxyl groups of the same or of two different chains. In the latter

case, a combination of the following type is theoretically produced:

Cellulose radical—O—CH<sub>2</sub>—O—cellulose radical

Stenosation actually produced products having an increased wet tensile strength and reduced swelling. However, this treatment can only be applied to finished products, and even then the conditions had to be maintained within very narrow limits in order to avoid formation of non-uniform or degraded products of little technical interest. Though stenosation increased the tensile strength of the product, nevertheless the elongation, resistance to friction and to knotting were greatly decreased. Additionally, the affinity of the product for dyes was materially affected irregularly and non-uniformly.

Another object of this invention is to provide a new and improved method of producing products obtained from solutions of cellulosic materials containing free hydroxyl groups.

A further object of this invention is to provide a method of producing synthetic shaped structures, such as yarns, filaments, fibers, bristles, foils, casings, tubings, films, caps, bands, etc., formed of a cellulose derivative.

Other and additional objects will become apparent hereinafter.

For sake of convenience, the invention will be described in connection with the production of yarns by the viscose process, though it is manifest that the invention is not restricted thereto.

The objects of this invention are accomplished, in general, by incorporating a resiniferous reagent, hereinafter more fully described, into a cellulosic solution and, after extruding the solution to produce a regenerated cellulose yarn of the desired shape and containing the reagent, causing the reagent by a thermal treatment to react with the cellulose whereby the cellulose is converted into a (relatively little) substituted derivative by forming bridge linkages between the cellulose chains. The resiniferous reagent contains bi- or poly-functional groups which will be converted into resiniform groups by polymerization, that is, high molecular weight groups obtained by linear bi-dimensional or tri-dimensional condensation.

The action of these bi- or poly-functional resiniferous reagents is similar to that of vulcanization agents in the rubber art, where isoprene chains greatly shortened during kneading are united to each other during vulcanization by bridge linkages formed by sulfur atoms.

The resiniferous reagents contemplated by this invention, moreover, should possess the following properties:

- (1) Be completely soluble in the spinning solutions;
- (2) Be stable in the presence of the constituents of the spinning solutions;
- (3) Have a sufficiently low molecular weight so as not to affect the viscosity appreciably;
- (4) Have a minimum effect on the index (or salt point) of the spinning solutions in order not to decrease the stability of the latter;
- (5) Precipitate out as completely as possible during coagulation of the spinning solution;
- (6) Not undergo any modification in reactivity under the influence of the coagulating baths;
- (7) Be practically insoluble in the finishing baths, and especially in the desulfurization bath;
- (8) Be capable of reacting with the hydroxyl groups of the cellulose;
- (9) Not degrade the cellulosic material.

The resiniferous reagents must be bi- or poly-functional in order to undergo polymerization or resinification. Moreover, during thermal treatment of the coagulated products suitably fixed by acid baths, there must be produced simultaneously with polymerization a reaction with the free hydroxyl group of the cellulose similar to etherification.

In general, the resiniferous reagent is a bi- or polymethyloxyaryl compound having the general formula:



wherein R is an aryl group, either cyclic or polycyclic, R' is an alkyl, aryl or acyl group or hydrogen, and n is at least 2. The radical R may comprise two or more phenyl groups combined

20 by direct saturation of their valences or by an oxygen, carbonyl, amine, hydrocarbon, etc. bridge or by polycyclic groups themselves united as explained above. Such reagents in the presence of heat, and preferably also in the presence of an 25 acid catalyst, react with cellulose material containing free hydroxyl groups to form resiniform bridge linkages by simultaneous polymerization (internal condensation) and etherification of the hydroxyl groups in the cellulosic material. The 30 cellulose derivative constituting the reaction product is herein termed "resyl cellulose" and probably has a constitution represented by the following general formula:

35 Cellulose radical—O—R—O—cellulose radical

wherein R designates a resiniform radical.

The reagents that have produced optimum results up to the present time are di- and trimethylolphenols obtained by reacting phenols with two 40 or three molecules of formaldehyde, in the form of Formol, per molecule of phenol preferably by the method of Manasse and Lederer (Berichte der deutschen chemischen Gesellschaft, 1894, vol. 27, p. 2409). These phenol alcohols preferably are slightly condensed, however not to the stage where they are in a resinous state. This condensation diminishes the solubility of the material in the coagulation bath in such a manner as to assure sufficient precipitation (of the order of 50 90%) during coagulation of the spinning solutions. However, condensation must be limited in such manner as to conserve the maximum number of active methylol groups, and the reagent must be completely soluble in dilute (from 55 5% to 10%) caustic soda aqueous solutions and ipso facto in viscose or other analogous alkaline solutions of cellulose derivatives.

When a different phenolic derivative is employed as the raw material, the poly-alcohol phenol is prepared in a similar manner to that previously described except that the quantity of Formol is determined by calculation of the maximum number of methylol radicals which can be fixed to the nucleus of the phenolic derivative used.

60 65 In carrying out the invention, the reagent is first prepared, then added in the desired quantity to the spinning solution, which is spun. After the yarn is fixed, it is subjected to the necessary liquid treatment, dried, and subjected to a thermal treatment, which may be included as part of the drying operation. It is during this latter treatment that the reaction between the reagent and the cellulose takes place.

The invention will now be described in greater 70 detail particularly for the case of the utilization

of polymethylolphenols, but, as has been mentioned above, it is not in any way limited to this case.

*Preparation of reagent*

Since it is necessary to use methylolphenols not polymerized in alkaline medium, the reaction is directed toward these products, avoiding the formation of resols. The condensation reaction is carried out in the presence of alkaline catalysts at a sufficiently low temperature so that the reaction will not be exothermic. Moreover, excess of formaldehyde should be avoided, that is, the quantity of formaldehyde should not exceed 3 molecules per molecule of phenol.

A solution of trimethylolphenol is prepared by known processes avoiding the formation of resin. This reaction may be carried out at temperatures of from 0° C. to 80° C. in the presence of alkaline catalysts (NaOH, CaO, etc.). Lower temperatures may be used by increasing the quantity of catalyst.

The phenol alcohol obtained is then subjected to polymerization carried out in acid medium in order to acquire the properties necessary for its incorporation in the spinning solutions. After neutralization of the alkali, it is heated for this purpose, but not to boiling, in the presence of weak acid catalysts having a pH of from 3 to 3.5 as a minimum.

Specifically, the neutralized liquid is rendered acid with concentrated lactic acid and is then heated at a temperature of from 96° C. to 98° C. for several hours. An emulsion forms after some time. Samples are taken and are washed with cold water. First, liquid products are obtained in this manner but, as condensation progresses, they become more and more paste-like. The operation is completed when the emulsion tends to "break," collecting at the bottom of the dispersed material. The free lactic acid is then neutralized with concentrated caustic soda carefully avoiding an excess of the latter and determining the pH after each addition.

Moreover, it was observed that the product must be absolutely free from free phenol and formaldehyde in order to avoid interferences in its utilization, namely, coloration of yarn, parasitic reactions, weakening of the yarn, etc. Also, salts must be eliminated. The product is washed several times with boiling water for this purpose. After cooling, an ivory-colored cake of pearly appearance is found at the bottom of the vat.

The reaction is practically quantitative under the described condition. The product finally obtained contains about 20% water. It is perfectly soluble in caustic soda up to concentrations of 50%. The stock solution thus obtained is stable on dilution, and the diluted solution poured into dilute sulfuric acid yields nearly quantitatively a white precipitate.

For utilization, a stock solution containing of the order of 50% of the trimethylolphenol in from 4% to 5% caustic soda is prepared and carefully filtered. This solution is also stable and may be stored for several days.

*Incorporation of the semi-condensed products into the spinning solutions*

The required quantity of stock solution is added to the spinning solution in such manner as to have present a ratio of from 1:10 to 1:1 of reagent to cellulosic material.

The incorporation of the stock solution into

the spinning solution is effected in such manner as to produce an intimate mixture rapidly.

If the mixture is made correctly, the salt point of the viscose is not affected (except slightly more rapid future evolution) and the variation in viscosity practically corresponds to that resulting from mixing two liquids having definite, determined viscosities. The desired viscosity may be obtained by suitable regulation of the viscosity of the viscose.

*Spinning*

The usual baths used in the viscose industry, such as the "Muller" type baths, are used for spinning viscose to which bi- or poly-functional resiniferous reagents have been added.

The metric number of filaments of the yarn does not seem to influence the amount of precipitation of reagent. No appreciable difference has been observed between yarns of filament No. 6000 and 900.

Spinning is not more difficult than in the case of the usual viscose and plugging of spinnerets is not increased if well-filtered stock solutions of reagent are used. It is advantageous to spin to a number in the neighborhood of 5, that is, the usual index.

*Fixation*

In order to obtain complete insolubility of the reagent precipitated in the heart of the regenerated cellulose, it is of advantage to maintain the yarn in an acid state for a certain period of time before submitting it to finishing, for example, for from 4 to 24 hours. However, this is not essential and in certain cases the yarn may be treated immediately as explained below, for example, in the case of continuous spinning.

*Finishing*

Desulfurization baths, such as the usual sodium sulfite baths, will be used but it is preferable to use baths which are only slightly alkaline in order to avoid losses by redispersion of the reagent.

Oiling is of great importance. In fact, some lubricating agents, such as sulfonated alcohols or polyamines, seem to favor definitely and to accentuate the action of the reagent on the cellulosic material. It may be supposed that these products, in reacting with the radicals forming resiniferous bridge linkages, for example, with the methylol groups not entering into reaction, accentuate the hydrophobic nature of the resin-form radicals. Similarly, softeners or plasticizers of the poly-alcohol type, such as glycerol, are capable of participating in the condensation reaction while conserving their activity. This fact is important in the manufacture of pellicles.

After oiling, the yarn is first dried as usual at from 90° C. to 100° C. After this drying, the hydrophobic nature of the yarn is not yet developed to a maximum, although considerable decrease in swelling is already observed.

It is pointed out that swelling is one of the properties determined by the conventional method and that the results obtained by this method have only a relative value. Primary swelling is herein defined as the weight of water retained by the yarn in percentages of the dry cellulosic material after thorough washing and centrifuging for 10 minutes in a centrifugal drier 25 cm. in diameter with 3,000 revolutions per minute. Secondary swelling is herein defined as the weight of water retained by the washed and dried yarn, which has then been rewetted and redried under the same conditions as previously.

Primary swelling for regenerated cellulose is usually of the order of from 150 to 200, and secondary swelling, of the order of from 100 to 120. For yarn obtained in accordance with the described process, secondary swelling is still of the same order or slightly lower after initial drying. However, it is greatly lowered by the second drying, or thermal treatment.

#### Thermal treatment

In principle, the yarn is later subjected to heating at from 100° C. to 115° C. or even higher, for a period of time varying with the temperature and in the presence of traces of weak acids. Acids having a dissociation constant of  $10^{-3}$  as a maximum change cellulose but slightly, and it is of advantage to use them in order to prevent degradation of the yarn. At a higher temperature, the duration of the thermal treatment may be shorter, and the quantity of acid catalyst smaller.

In the case of yarn, heating may, for example, be carried out in a chamber at from 115° C. to 120° C. for from 2 to 3 hours at a pH of from 4 to 4.5 resulting from the addition of from 1 to 2 grs. of lactic acid or acetic acid to the oiling bath. If desired, the yarn may also be impregnated with a catalyst.

The thermal treatment may also be carried out continuously at a higher temperature, such as of the order of from 130° C. to 140° C., at the same pH, by passage over heated rolls.

Moreover, it is not essential that the thermal treatment immediately follow the usual finishing treatments. The yarn may be converted to manufactured products (fabrics, knit goods, etc.) and the thermal treatment thereafter applied to such manufactured products.

Whereas a temperature of from 115° C. to 120° C. seems necessary when using organic catalysts, a lower temperature may be used in the presence of stronger acids.

The resiniferous reagents to be added to the spinning solutions may be combined with other suitable products, particularly with other polymerized and etherifiable substances capable of reacting with the complex formed and capable of forming new complexes. Polyvinyl alcohol or its derivatives, polyglycerides, or polymerization products of acetic aldehyde may be used. These substances may be introduced into the alkaline solution either directly or in the form of xanthogenate or other derivatives. Also, resins or their conversion products, dyes, delustering agents, pigments, plasticizers, etc. may be added to the resiniferous reagents.

The examples herinafter described are illustrative embodiments of the invention, but it is obvious that these examples are in no way limitative of the scope of this invention.

#### Example 1 (manufacture of continuous filaments)

To a viscose solution containing 7% cellulose and 6% caustic soda were added 4% of a stock solution of 60 grs. per liter of caustic soda and resiniferous material of the trimethylolphenol type, prepared as indicated above. Viscose prepared in this manner contained 19% of dry reagent based on the cellulose. After ripening up to a salt point of 5, this viscose was spun through a spinneret having 1000 orifices, into a bath containing 130 grs. of sulfuric acid, 250 grs. of sodium sulfate, and 10 grs. of zinc sulfate per liter at a speed of 80 meters per minute, forming a product of metric number 5. The yarn was washed and then desulfurized with a sodium sulfite solution at

60° C. Thereafter, it was oiled with a solution containing a product known by the trade name "Soromine AF" (a fatty acid derivative—see Textil-Hilfsmitteltabellen, Berlin, 1938, p. 260) and 1 gr. of lactic acid per liter, and dried at 90° C. The dried product was then subjected to a temperature of 115° C. The product thus obtained had a swelling of 40.

#### Example 2 (manufacture of bristles)

To a viscose solution containing 7% cellulose and 6% caustic soda prepared from a slightly ripened or unripened alkali cellulose having a viscosity of the order of 120 centipoises, were added 6 parts of the aforementioned stock solution per 1 part of viscose. The viscose obtained in this manner contained about 32% of dry reagent with respect to the cellulose. It was spun in a coagulating bath containing 80 grs. of ammonium sulfate and 40 grs. of sulfuric acid per liter, at a temperature of 40° C. and with a spinneret having a single orifice of 0.2 mm. at a rate of 30 meters per minute. A bristle of metric number 15 was obtained and was fixed in a bath containing 120 grs. of sulfuric acid per liter, at room temperature. It was then washed with water and finally with a 2% solution of ammonium acid phosphate. It was dried at 90° C. and then treated at 115° C. for 2 hours. The swelling of the bristle was 42.

#### Example 3 (manufacture of thin pellicles)

To a viscose solution, similar to that of Example 1, were added 4 parts, per 100 parts of viscose solution, of the stock solution of condensed trimethylolphenol, and then 6 parts of a 15% aqueous alcoholic solution of polyvinyl butyral xanthogenate per 100 parts of viscose solution. The solution was ripened to a salt point of 2, then cast by means of a hopper into a bath containing 120 grs. of sulfuric acid and 200 grs. of sodium sulfate per liter. The resulting pellicle was suitably washed and desulfurized, as in Example 1, and was treated with glycerol in an aqueous bath containing 10% glycerol and also more than 2 grs. per liter of lactic acid. It was dried on a drum at a final temperature of 125° C. The finished pellicle had a swelling of 45 and was quite insensitive to water.

#### Example 4 (manufacture of fiber with a high resiniform radical content)

A viscose solution, containing 7.5% of cellulose and 6.5% of caustic soda and having a salt point of 5.5, was mixed with 18% of a stock solution of pre-condensed reagent, resulting in a content of about 90% of reagent with respect to the cellulose. The mixture was spun immediately at a rate of 70 meters per minute, using a spinneret having 2500 orifices. The product, while in an acid state, was cut into pieces (staple), then washed and desulfurized, oiled as in Example 1, dried at 90° C., and finally treated at 115° C. for 2 hours. The fiber obtained in this manner had a swelling of 30. It was slightly yellowish, but was distinguished from ordinary fiber by its spring, that is, its resistance to crushing (and creasing).

In order to determine this crush resistance, a given weight of fiber was placed in a vessel, a weight (for example 5 kg.) was placed on it, and the weight then removed. The fiber of the present example returned to such a point that its final volume was 4 times greater than in the case of ordinary fiber.

In general, the products of the invention swell only to the extent of 40% to 50%, or even less, of that of comparable products of ordinary regenerated cellulose. It is to be noted that the products obtained according to the present invention are not weakened in any way by the thermal treatment if the latter is not exaggerated. Some of the results of tensile strength measurements obtained for fiber made in accordance with the invention, but with thermal treatments of different duration, are given in the following table:

|                                  | Kilometric<br>dry<br>strength | Kilometric<br>Strength<br>Ratio,<br>Wet:Dry | Elasticity |     |
|----------------------------------|-------------------------------|---------------------------------------------|------------|-----|
|                                  |                               |                                             | Dry        | Wet |
| Unpolymerized yarn               |                               |                                             | Per cent   |     |
| Treatment for 6 hours at 105° C. | 16.6                          | 0.81                                        | 29         | 31  |
| Treatment for 2 hours at 120° C. | 16.8                          | 0.84                                        | 29         | 32  |
| Treatment for 1 hour at 138° C.  | 16.7                          | 0.81                                        | 30         | 31  |
|                                  | 16.8                          | 0.82                                        | 26         | 26  |

There are extremely numerous and varied applications of the invention. The decrease in secondary swelling of regenerated cellulose is of considerable interest in all the fields of application of regenerated cellulose products. As was mentioned above, the invention is applicable to the manufacture of yarn, threads, filaments, bristles, foils, casing, tubing, caps, bands, etc. The new cellulose derivatives, in accordance with the invention, are characterized primarily by their slight swelling. The latter, however, corresponds to a reduced sensitivity to water, steam, and to the variations in the relative humidity of the air. The wet strength of products of these new cellulose derivatives is high. Whereas in the case of artificial yarn of regenerated cellulose, the ratio between the wet and dry strength is usually of the order of from 45% to 50%, it is 60% or more for artificial yarns made in accordance with the invention. At the same time, the dry strength is increased more or less.

The artificial yarn of the invention is also characterized by substantially no shrinkage on wetting, even with slightly alkaline aqueous liquids at boiling, such as washing liquors. Shrinkage on washing is one of the serious defects of artificial yarn and especially staple fiber articles, the dimensions of which may decrease under certain conditions from 10% to 25%, rendering the articles non-useable.

Articles of natural textiles, such as cotton, wool, etc., are not immune to the mentioned defect, and one of the great advantages of the invention is to make possible the manufacture of knit goods and fabrics, etc., the dimensions of which are not in any way affected by washing, laundering, etc. even under rigid conditions. Moreover, unlike woolen fabrics, fabrics of artificial yarn, in accordance with the invention, do not felt when treated with aqueous liquids at boiling. Thus, squares of fabric made from fiber obtained according to the invention and treated for 15 minutes by boiling in a solution containing 5 grs. of Marseilles soap per liter, show a negligible decrease in length and width, whereas squares of wool of identical texture were completely deformed and felted after an identical treatment.

Yarn made according to the invention, in the form of rayon and staple fiber, has an absolutely remarkable spring and resists crushing and

creasing much better than ordinary artificial textiles. Elasticity on creasing and twisting is greatly increased. The articles, knitted fabrics, etc. made from yarns of the invention have a much better appearance than those made of ordinary artificial yarns. On the other hand, their "nervous" feel enables them to compare favorably with natural textiles, especially wool.

Unlike artificial yarns obtained by application of stenosation, the affinity for dyes is generally not diminished and, on the contrary, dyeing in the case of certain direct dyes is facilitated and uniformity improved. Yarns made according to the invention even possess a certain affinity for dyes for cellulose acetate, clearly indicating that here it is a matter of cellulose derivatives and not mixtures of cellulosic materials and resinous materials. It is to be noted that increase of the affinity for dyes is only manifested if the decrease in swelling is not carried to an excessive degree. In the latter case, a decrease in dye affinity may result.

The minimum sensitivity to humidity of yarns made according to the invention facilitates their conversion into knitted articles and fabrics. It is well known, in fact, that in converting regenerated cellulose yarns, the relative humidity of the air of the rooms must be maintained rigorously constant in order to avoid irregularities in the fabric. In making yarn from staple fiber of regenerated cellulose, precaution must be taken to assure sufficient uniformity of the yarn. This factor is much less important for staple fibers of the invention, since they are only slightly sensitive to humidity. Irregularities in tension during spinning are also less dangerous.

Moreover, textile articles made of yarns of the invention are wetted with much more difficulty than articles of ordinary artificial yarns and are not only comparable to articles of wool but also are even superior to them. On wetting, the drops slide without really wetting, and a long "wetting time" is necessary before the article is really wetted. Consequently, and also because of the smaller deformation on wetting, the serious defect of deformed regions, manifested, for example, by fabrics of rayon or fiber of ordinary viscose, is eliminated completely.

Bristles (which are usually monofilament) made according to the invention are extremely interesting. Whereas bristles of regenerated cellulose, known up to the present, and even analogous bristles having a resin treatment were never suitable for brushes because of their very poor behavior on bending, rubbing, etc., the bristles made according to the invention behave very favorably and advantageously replace animal bristles, to which they are even superior because of their great regularity. The modulus of elasticity is double or more of that of regenerated cellulose bristles, and the bending (folding) resistance is also much better. Bristles made according to the invention also compare favorably with artificial resin bristles and polymerized products in general, over which they also have the advantage of much lower cost.

The small sensitivity to water of the bristles and also of foils made from cellulose derivatives according to the invention makes possible even greater application of these products in the millinery industry and other branches of the fashion-articles industry where deformation on wetting was a disadvantage.

The great swelling in water and ease of wetting 75 of thin pellicles of regenerated cellulose were a

great disadvantage in the use of these pellicles in certain industries where they could have found a considerable market. Attempts have been made to overcome this by lacquering, coating, or other surface treatments. However, excluding the difficulties involved in carrying this out and the additional complications in the normal manufacturing process caused thereby, there is a serious question of cost, since such treatment increases the price considerably. The present invention makes it possible to obtain thin pellicles of regenerated cellulose which have very much reduced swelling properties, small sensitivity to wetting, are extremely flexible, and slightly permeable to vapors of water and solvents. These pellicles are suitable not only in numerous applications, as wrappings for products sensitive to humidity, such as cigarettes, sugar products, pastries, etc., but are also very interesting as wrappings which must withstand the low temperatures of refrigerating plants. The latter application requires products having good resistance to wetting, being slightly permeable to water vapor and being able to remain at low temperatures frequently. All these qualities are present in the pellicles made in accordance with this invention.

The pellicles of this invention may also be used advantageously in photography, motion pictures, sound recordings, etc., where regenerated cellulose pellicles have been used. They also can be used industrially, whereas the prior art regenerated cellulose pellicles, because of their great sensitivity to water and water vapor, could not be used. In fact, water and water vapor produce more or less great deformation of pellicles, and hence of the pictures or other recordings, and affect the quality of the reproduction. The pellicles of this invention, much less sensitive to water, are thus in a position to find very interesting applications in these industries, especially in combination with sensitization in the mass, producing images and recordings without visible opacity.

Pellicles made according to the invention are also of interest in other fields. Thus, they may be cut into foils and fiber and used in making fashion articles which will be considerably less sensitive to water than known articles. These pellicles may also be used as membranes in dialysis because of their excellent resistance to water and even to alkaline and acid liquids.

The process of the invention also lends itself to the manufacture of artificial casings which must have a sufficient wet strength to resist stuffing with sausage meat. Caps and bands for applications requiring rapid drying are also within the scope of the invention.

Certain additional applications in the field of molded products may be considered, where deformation or drying was of disadvantage in the industrial application of cellulose.

The invention is applicable not only to regenerated cellulose, but also more generally, as has been previously explained, to various products obtained by spinning, molding, etc., from solutions of cellulose derivatives containing free hydroxyl groups. In particular, it has very interesting applications in the case of certain cellulose derivatives which are easy to prepare and present certain advantages over cellulose xanthogenate from the point of view of facility and economy of conversion. These cellulose derivatives, namely hydroxyalkyl- or glycol-cellulose, cellulose carboxylic acids, slightly substituted methyl and ethyl celluloses, have an excessive swelling, and products made from their solutions in general

have a low resistance, and especially a low wet strength. The incorporation of the aforementioned resiniferous compounds into their alkaline solutions, combined with thermal treatment of the finished products, results in products having greatly improved properties and capable of finding extremely interesting applications.

The invention may also be applied in combination with other processes of spinning solutions of cellulose derivatives. In the case of dry spinning, the trimethylolphenols may be used directly without precondensation, the possibility of loss of reagent in precondensation not existing, while drying assures sufficient precondensation to permit of finishing treatments without excessive losses.

In the case of pot spinning, with drawing by mobile fluids, of a superficially coagulated filament, it is essential to use precondensed products. More especially, in the case of viscous spun in this manner, slightly acidified baths are used in combination with greatly ripened viscose, the slight acidity of the bath being sufficient to precipitate most of the reagent.

The process of the present invention differs from known processes in which more or less soluble resols or resins which do not react with the hydroxyl groups of cellulose and form an inert mass within the cellulosic material are dispersed in the spinning solutions. The object of such known processes was either to modify the affinity for dyes of the cellulosic material, or to fix mechanically impressed designs on the spun material, or to decrease shrinkage on washing, or even to impart to the cellulosic material less absorbent properties. However, the decrease in swelling which may be achieved in this manner is much less significant than that obtained by the process of the present invention. It is to be noted in this connection that in using reagents in accordance with this invention the activity varies with the importance of the functional groups which enter into reaction.

As was stated above, the addition of various condensation products of phenol and formaldehyde to the spinning solutions has previously been suggested. In numerous patents it was suggested especially to use the condensation products of one molecule of phenol with approximately one molecule of formaldehyde, such products in principle being condensed in alkaline medium at boiling, and forming products of the resol type and containing no, or practically no, free methylol functions. The object and effect of adding these products to spinning solutions were improvement of dyeing properties of the yarn as well as fixation of printing, and, to a certain extent, the resistance to wetting of the fibers of regenerated cellulose by blocking its pores without modifying the chemical properties of the cellulose.

It was also suggested to eliminate the disadvantages of coloration of phenolic compounds under the influence of light by using condensation products obtained from 1 molecule of phenol and 3 molecules of formaldehyde or more in alkaline medium and also at boiling. Products of the type of high molecular weight resols were obtained, having only a fraction of their methylol groups in a free state and, consequently, no longer having any etherifying ability for the cellulosic hydroxyl groups. In addition, such processes included polymerization of these phenolic products during or after drying of the yarn by applying suitable temperatures, but either in the presence of alkali which served as catalyst for con-

densation, or in neutral medium, and in all cases never in acid medium which is the essential condition for obtaining etherification of the cellulosic hydroxyl groups of methylol groups. Finally, the number of methylol groups of these compounds was decreased considerably by resinification of the initial products.

The reagents in accordance with the invention are clearly defined by their chemical properties. In addition to the new chemical properties acquired by the yarn, the formation of a compound between regenerated cellulose and the reagent incorporated into the spinning solution is proved by the fact that the tensile strength of the yarn only differs very little from the corresponding property of yarn obtained in the absence of these reagents. In fact, as a general rule, any addition of foreign substances to spinning solutions (the charge, delustering agents, resins, protein substance, etc.) is manifested by a more or less great decrease in tensile strength and elasticity. This is not so for products in accordance with this invention. According to this invention, artificial yarn may be produced using very large quantities of reagents (for example, from 40% to 50%) without diminishing tensile strength, the yarn being even strengthened by 20% in the dry state and 40% or more in the wet state. The resultant products are not heterogeneous mixtures and the added reagents combine chemically with the cellulosic material. The phenomena of plastic flow manifested during drawing of the yarn are diminished and the modulus of elasticity increased.

In copending application Serial No. 649,777, filed on even date herewith, now Patent Number 2,495,233, there is disclosed, in general, resyl cellulose and the preparation thereof from any cellulosic material. In copending application Serial No. 649,779, filed on even date herewith, now Patent No. 2,495,233, there is disclosed a process wherein already-prepared articles especially of regenerated cellulose, and such as yarns, filaments, bristles, films, etc., are converted to resyl cellulose.

Since it is obvious that various changes and modifications may be made in the above description without departing from the nature or spirit

thereof, this invention is not restricted thereto except as set forth in the appended claims.

We claim:

1. A method of producing from cellulosic material shaped structures which show improved resistance to swelling, which comprises dissolving in a viscose spinning solution a non-resinous slightly condensed polymethylolphenol reagent capable of forming resiniform bridge linkages between cellulose chains and consisting essentially of a trimethylolphenol, extruding said spinning solution in the shape of the desired structure in an acid bath which co-precipitates both the cellulosic substance and the polymethylolphenol from said spinning solution, and subjecting the structures to finishing treatment which includes thermal treatment to produce a resinification of the bridge linkages between the cellulose chains by the reaction of the hydroxyl groups of the cellulosic material with the polymethylolphenol.
2. A spinning solution consisting of an aqueous alkaline solution of cellulose xanthate and a non-resinous slightly condensed polymethylolphenol reagent capable of forming resiniform bridge linkages between cellulose chains and consisting essentially of a trimethylolphenol.

NICOLAS DRISCH.  
RENE FAYS.

#### REFERENCES CITED

The following references are of record in the file of this patent:

#### UNITED STATES PATENTS

| Number       | Name            | Date           |
|--------------|-----------------|----------------|
| 2,054,444    | Pinten          | Sept. 15, 1936 |
| 2,190,672    | Mehang          | Feb. 20, 1940  |
| 2,229,357    | Wightman et al. | Jan. 21, 1941  |
| 2,288,695    | Fuller          | July 7, 1942   |
| 40 2,315,400 | D'Alelio        | Mar. 30, 1943  |
| 2,322,981    | Ubbelohde       | June 29, 1943  |
| 2,360,376    | Van Epps        | Oct. 17, 1944  |

#### OTHER REFERENCES

45 Granger, Condensation of Phenols with Formaldehyde, Ind. and Chem., April 1932, pages 442 and 447.